

W. G. MICHEL,

PROCESS AND APPARATUS FOR MAKING ELECTRODES.  
APPLICATION FILED DEC. 17, 1919.

1,378,599.

Patented May 17, 1921.



WILLIAM G. MICHEL

Inventor

By Frank Keifer

Attorney

# UNITED STATES PATENT OFFICE.

WILLIAM G. MICHEL, OF NIAGARA FALLS, NEW YORK.

## PROCESS AND APPARATUS FOR MAKING ELECTRODES.

1,378,599.

Specification of Letters Patent. Patented May 17, 1921.

Application filed December 17, 1919. Serial No. 345,659.

To all whom it may concern:

Be it known that I, WILLIAM G. MICHEL, a citizen of the United States, residing at Niagara Falls, in the county of Niagara and State of New York, have invented certain new and useful Improvements in Processes and Apparatus for Making Electrodes, of which the following is a specification.

The object of this invention is to provide new and improved forms of electrodes and abrasives and a process for making them.

This and other objects of the invention will be fully illustrated in the drawings, described in the specification and pointed out in the claims at the end thereof.

In the accompanying drawings,

Figure 1 is a diagrammatic view of the apparatus for making the electrodes.

Fig. 2 is a view of the tube or mold in which the electrode or abrasive is made.

In the drawings, like reference numerals indicate like parts.

It will be understood that electrodes have heretofore been made of pulverized coal, or graphite, or coke, or charcoal, or other suitable conductors that are more or less proof against corrosion by electrolytes. These electrodes must be formed to certain desirable shapes and can best be formed in those shapes by reducing the conducting material of the electrode to small pieces or pulverized condition and compressing them together and then binding these pieces together by a suitable binder, such as tar, pitch, oil or shellac, which binding material is ordinarily non-fluid or congealed when cold and is in a fluid condition when hot. This process must also be followed in preparing abrasives such as hones, polishing or grinding wheels and the like.

In preparing electrodes, I therefore take the desired conducting material and reduce it to the proper condition of fineness and compress it in the desired form into a suitable receptacle. I then bring the binder into intimate contact therewith under conditions of suitable temperature and pressure so as to secure an intimate mixture of the binding material with the conductor so that cohesion between them will be properly and effectively secured. For the purpose of this heat and pressure treatment I provide the following apparatus.

In the drawings, reference numeral 1 indicates an elevated tank in which an agi-

tator 2 is mounted to move to stir up and mix the ingredients that are contained in the tank. In this tank is placed the binding material for the electrodes, which binding material will depend upon the use to which the electrode will be put and consists of either tar, pitch, oil or shellac or a combination of them. The tank 1 is heated and the agitator operates to mix and secure the even heating of the materials therein until it is reduced to a suitable fluid consistency. After this is done, the fluid is drained off through the pipe 3 into the reservoir 4 which is also heated in order to keep the contents in a liquid state.

The material for the electrodes is formed in suitable forms or molds such as pipes having one end thereof closed and the other end open. One of these forms indicated by the reference numeral 5 is shown in Fig. 75 2. The material for the electrode such as pulverized coal or graphite or coke or charcoal, is placed in the pipe or mold. It will be understood that a great variety of shapes may be used for this purpose.

A number of these molds are filled with the proper ingredients, and they are then placed in a boiler 6 in an upright position therein, a man hole 17 being provided in the boiler for this purpose.

After a suitable number of molds has been placed therein the boiler is hermetically sealed and the air is exhausted therefrom by a vacuum pump through a pipe line 7, in which pipe line is placed a trap 90

8. After a suitable vacuum has been created in the boiler 6, the valve 9 is opened permitting the fluid binder contained in the reservoir 4 to flow or be drawn into the boiler 6 and fill it. The fluid binder flows 95 into the molds and fills the interstices between the powdered particles forming the material for the electrodes, which fluid because of the previous partial vacuum, will readily fill these interstices. After the oil has filled the boiler and has impregnated the electrodes, pressure may be applied to it to make it the more completely impregnate the electrodes. For this purpose, the valves 10 and 11 are closed and the valves 100 12, 13 and 9 are left open and air pressure is then applied to the boiler 6 from the storage tank 14. This causes the fluid to fill the forms under pressure and more completely penetrate the interstices in the elec-

70

75

80

85

90

95

100

105

110

trodes. A gage glass 20 is provided which shows the level of the binder in the boiler so that the correct amount may be supplied to the boiler. This glass will also show 5 when the absorption of the binder by the electrodes has been completed.

After the filling of the electrodes has been completed, the valves 9 and 12 are closed and the valve 15 is opened and the air pressure from the tank 14 will cause the fluid to flow through the pipe 16 to the agitator tank 1, emptying the boiler 6. The air pressure is kept on and the boiler is kept heated in any suitable manner for four hours or 10 more, after which the binder is again admitted and the pressure is applied and the above treatment is repeated after the excess binder has been finally expelled. It will also be understood that the reservoir and 15 agitator tank will be kept heated in any suitable manner as by steam coils or electric conductors. The man-hole 17 may then be opened and the molds containing the electrodes may be removed after which the 20 molds are placed in an oven or furnace and are subjected to a high temperature causing the baking of the electrodes. After the electrodes have been baked sufficiently to make them hard, they can be removed from 25 the forms and are ready for use.

It will be understood that the tank 1, the reservoir 4 and the boiler 6 are kept constantly heated in order to keep the binding material in a liquid state. The air storage tank 14 may also be heated so that the fluid binder will not be chilled by cold air being allowed to come in contact with it.

For the purpose of heating the binder, steam heat is used, the steam being at a 40 pressure of about 80 lbs. with a corresponding temperature.

The air pressure which is used for forcing the binder into the electrodes may be anywhere from about 125 lbs. to as much as 45 1,000 lbs. or even higher.

For making a graphite electrode, I prefer a binder which is made of 25% crude oil and 75% coal tar. For coke electrodes, I prefer a binder made of 50% pitch and 50% 50 coal tar. For coal electrodes, I prefer from 25% to 33½% crude oil and 66½% tar. For charcoal electrodes, I prefer 75% coal tar and 25% kerosene oil. For abrasive, such as emery and carborundum, for the purpose 55 of forming stones or hones or wheels therefrom, and more especially where the wheels are coarse and slow running, I prefer a binder made of 100% pitch or tar. For high speed wheels I prefer 100% shellac, it being

60 understood that the same process that is used for making electrodes is also used for making abrasive stones or abrasive wheels, the binder being selected in each individual case.

65 It will also be understood that some of

these electrodes are to be used in the presence of chemicals and the binders must be such as will resist chemical action therefrom and other electrodes will be used exposed to heat and the binder must be such as will resist 70 the effect of heat.

I claim:

1. An electrode composed of pulverized dry carbon, the particles of carbon being held together by a fluid hydrocarbon mixed 75 therewith and baked to a solid mass, said fluid being heated and mixed with the carbon by vacuum and pressure.

2. The process of making electrodes which consists of (1) reducing the material for the 80 electrode into powdered form, (2) filling suitable molds with said powdered material, (3) exhausting the air which occupies the interstices between the powdered particles by subjecting the mold and its contents to 85 a partial vacuum, (4) filling the voids created by the partial vacuum between the powdered particles in the mold with a liquid binder, said liquid binder being forced into the mold under pressure.

3. The process of making electrodes which consists of (1) reducing the material for the electrodes into powdered form, (2) filling suitable molds with said powdered material, (3) placing the filled molds into a hermetically sealed boiler, (4) exhausting the air from said boiler surrounding said molds in order to exhaust the air filling the interstices between the powdered particles, (5) introducing a liquid binder into the partial 100 vacuum created between the powdered particles, (6) forcing said liquid binder between the interstices of said powdered particles.

4. The process of making electrodes which consists in forcing a liquid binder into the 105 powdered electrode material by means of pressure.

5. The process of making electrodes which consists in exhausting the air that separates the powdered particles forming the electrode 110 material from one another and then allowing a binder in its liquefied form to occupy the voids thus created between the powdered particles.

6. The process of making electrodes which 115 consists in exhausting the air that separates the powdered particles forming the electrode material from one another and then allowing a binder in its liquefied form to occupy the voids thus created between the powdered 120 particles, air pressure being used to unite the binder with the powdered particles to form a homogeneous mass.

7. The process of making electrodes which 125 consists of (1) filling suitable molds with powdered electrode material, (2) exhausting the air from between the interstices of said powdered material in said mold, (3) introducing a liquid binder into said mold to fill the interstices between said powdered mate- 130

rial, (4) compressing said powdered material with said liquid material by means of compressed air introduced into said mold.

8. The process of making electrodes which  
5 consists of (1) filling suitable molds with powdered electrode material, (2) exhausting the air from between the interstices of said powdered material in said mold (3) introducing a liquid binder into said mold to fill

the interstices between said powdered material, (4) compressing said powdered material with said liquid material by means of compressed air introduced into said mold, (5) the application of heat to the outside of the mold after the powdered material and 15 its binder have been compressed.

In testimony whereof I affix my signature.

WILLIAM G. MICHEL.